

## 1

3,108,958

LUBRICANT ADDITIVE AND COMPOSITION  
CONTAINING SAME

Donald L. Klass, Barrington, Ill., and Roger W. Watson, Highland, Ind., assignors to Standard Oil Company, Chicago, Ill., a corporation of Indiana  
No Drawing. Filed Dec. 8, 1958, Ser. No. 778,576  
11 Claims. (Cl. 252—32.7)

This invention relates to additive compositions for use in lubricating oils, the use of such additive compositions, and improved lubricating compositions containing such additive compositions and intended for use in internal combustion engines such as diesel engines and automobile engines. More particularly the invention relates to additive compositions which impart detergency and anti-rust properties to lubricating oils and suppress excess varnish formation when used in lubricating oils.

Straight petroleum lubricants are effective within certain defined limits of engine operating conditions and when these limits are exceeded, such lubricants frequently fail to give the desired performance demanded of them. Since, in modern engines designed to give increased performance, these limits are frequently exceeded, the use of straight mineral oils as lubricants produce undesirable conditions within the engine; thus varnish formation and corrosion are excessive in modern engines using mineral oils alone.

It is an object of the present invention to provide a new composition for use as a lubricant additive. It is another object to provide a lubricating oil additive composition which imparts detergency, anti-varnish formation and anti-rust properties to a lubricating oil. It is a further object of the present invention to provide a lubricating oil having these properties and suitable for use in a modern internal combustion engine. Other objects and advantages of our present invention will be apparent from the descriptions and examples set out below.

We have discovered that a hydrolyzed phosphorus sulfide-hydrocarbon reaction product may be reacted with an amine compound and a fluoroboric acid such as difluoroboric acid to form a new composition of matter with desirable characteristics for use as an additive composition in a lubricating oil. When used in a lubricating oil in even very small amounts, i.e. in amounts as low as 0.1 wt. percent and preferably not exceeding 20 wt. percent, the boron, fluorine and amine-containing additive composition of our present invention overcomes the problems of the mineral lubricating oil in its use without additives by imparting to the lubricating oil high detergency properties and eliminating excessive varnish formation and corrosion. The new additive may also be used in an additive concentrate in amounts of from 10 to 50 weight percent or more for addition to lubricating oils.

Broadly, our present invention provides an additive composition for lubricating oils formed by reacting a hydrolyzed phosphorus sulfide-hydrocarbon reaction product with at least a sufficient amount of an amine compound to neutralize the reaction product and then reacting the resulting neutralized reaction product with a fluoroboric acid such as difluoroboric acid and monofluoroboric acid. Our invention also provides an improved mineral oil containing an effective amount of our additive composition to impart improved properties to the lubricating oil.

The amine compound used in preparing the additive composition of our present invention may be any aliphatic or substituted aliphatic compound having 1 or more basic amine groups. Preferred amine compounds particularly suited for use in the preparation of the additive composition of our present invention are the hydroxy aliphatic amines such as monohydroxy, dihydroxy, and polyhy-

## 2

droxy aliphatic amines and particularly preferred are the aliphatic polyamines such as diamines, triamines, etc., having two or more carbon atoms in the aliphatic chain. Polyhydroxy aliphatic polyamines are includable in either group. Particularly suitable aliphatic polyamines are alkylene polyamines containing at least two primary amino nitrogen atoms. Examples of alkylene polyamines suitable for the herein-described purpose are ethylene diamine, propylene diamine, diethylene-triamine, diamylene triamine, triethylene tetramine, tripropylene tetramine, diethylene-propylene tetramine, tetraethylene pentamine, tetrabutylene pentamine, diethylendipropylene pentamine, butylene diamine, dihexylene triamine, and the like, or mixtures thereof. For example, a suitable polyamine product is a crude diethylene triamine containing minor amounts of ethylene diamine and triethylene tetramine. Other suitable aliphatic polyamines include those having the general formula  $RNH(CH_2)_3NH_2$ , in which R is preferably a  $C_{10}$  to  $C_{18}$  aliphatic chain, and which are obtained by condensing the suitable amine with acrylonitrile and hydrogenating to the corresponding diamine. Commercially available aliphatic polyamines of this type are those marketed by Armour and Company as "Duomeens," which are prepared by the condensation of a dodecyl (coco) amine or an octadecyl (tallow) amine with acrylonitrile followed by hydrogenation to the corresponding diamine product; these products are marketed as "Duomeen C" and "Duomeen T," respectively.

The difluoroboric acid, a liquid, may be conveniently prepared by reacting  $B_2O_3$  with hydrogen fluoride as taught by F. J. Sowa et al., JACS 57,454 (1935).

The hydrolyzed phosphorus sulfide-hydrocarbon reaction product may be prepared by any method known to the prior art. We prefer to react a hydrocarbon with oil from about 1% to about 50%, and preferably from about 5% to about 25% of phosphorus sulfide at a temperature of from about 200° F. to about 600° F. in a non-oxidizing atmosphere, as, for example, in a nitrogen atmosphere. The reaction is carried out for from about one to about ten hours or more, and preferably for about five hours. The reaction may be carried out in the presence of a sulfurizing agent such as sulfur, sulfur chlorides, etc., if desired. The product is hydrolyzed at a temperature of from about 200° F. to about 500° F., and preferably at a temperature of from about 220° F. to about 400° F. by hydrolyzing means, for example, by introducing steam through the reaction mixture. The hydrolyzed product may be solvent extracted to remove salts of inorganic phosphorus acids and low molecular weight organic phosphorus acids formed during hydrolysis. Solvent extraction may be accomplished in accordance with the method described by Norman E. Lemmon et al. in U.S. 2,843,579, issued July 15, 1958.

In the phosphorus sulfide-hydrocarbon reaction used for preparing starting materials for the additive compositions of the present invention, any phosphorus sulfides such as  $P_4S_3$ ,  $P_4S_7$ ,  $P_4S_{10}$ , or other phosphorus sulfides and preferably phosphorus pentasulfide,  $P_2S_5$ , may be reacted with a hydrocarbon.

The hydrocarbons used in the phosphorus sulfide-hydrocarbon reaction may be polymers such as mono-olefin polymers, copolymers, graft polymers, etc. and may also be unpolymerized or unpolymerizable hydrocarbons such as olefins, paraffins, cycloparaffins, aromatic hydrocarbons, etc.

The mono-olefin polymer to be treated may be the polymer resulting from the polymerization of low molecular weight mono-olefins preferably the isomono-olefins, such as isobutylene and isoamylene and/or the copolymers obtained by the polymerization of hydrocarbon mixtures containing isomono-olefins and mono-olefins of less than six carbon atoms and preferably those of four carbon

atoms. The polymer may be obtained by the polymerization of these olefins or mixed olefins in the presence of catalysts such as sulfuric acid, phosphoric acid, or boron fluoride, aluminum chloride or other similar halide catalysts of the Friedel-Crafts type. The polymers advantageously have molecular weights ranging from about 150 to about 50,000 or more, and preferably from about 500 to about 10,000.

Various polymerized starting materials prepared by methods well known in the art may be used. For example, as a starting material there can be used the polymer or synthetic lubricating oil obtained by polymerizing the unsaturated hydrocarbons resulting from the vapor phase cracking of paraffin waxes in the presence of aluminum chloride which is fully described in U.S. Patents Nos. 1,955,260; 1,970,402; and 2,091,398. Still another type of olefin polymer which may be employed is the polymer resulting from the treatment of vapor phase cracked gasoline and/or gasoline fractions with sulfuric acid or solid adsorbents, such as fuller's earth, whereby the unsaturated polymerized hydrocarbons are removed. Also contemplated within the scope of this invention is the treatment with phosphorous sulfide of the polymers resulting from the volatilization of hydrocarbons as described for example in U.S. Patents Nos. 2,197,768 and 2,191,787.

Other hydrocarbons which we can use as reactants in the preparation of the phosphorus sulfide reaction product are paraffins, olefins, aromatics or alkyl aromatics, cyclic aliphatics, petroleum fractions, such as lubricating oil fractions, petrolatums, waxes, cracking cycle stocks, condensation products of the foregoing hydrocarbons, solvent extracts of petroleum extracts, etc.

The paraffin hydrocarbons can be those obtained from petroleum oils such as bright stock residuums, lubricating oil distillates, petrolatums, or paraffin waxes. We may also halogenate any of the foregoing paraffins and condense the same with aromatic hydrocarbons in the presence of anhydrous inorganic halides such as aluminum chloride, zinc chloride, boron fluoride and the like.

As examples of high molecular weight olefinic hydrocarbons which we may employ as reactants are cetene ( $C_{16}$ ), cerotene ( $C_{26}$ ), melene ( $C_{30}$ ) and mixed high molecular weight alkenes obtained by cracking petroleum oils.

Other preferred olefins suitable for the preparation of the herein described phosphorus sulfide reaction products are olefins having at least 20 carbon atoms in the molecular of which from about 13 carbon atoms to about 18 carbon atoms, and preferably at least 15 carbon atoms in a long chain. Such olefins can be obtained by the dehydrogenation of paraffins, such as by the cracking of paraffin waxes or by the dehalogenation of alkyl halides, preferably long chain alkyl halides, particularly halogenated paraffin waxes.

As further examples of starting materials for the preparation of the hydrolyzed phosphorous sulfide-hydrocarbon, any of the hydrocarbons recited as useable by Norman E. Lemmon et al. in U.S. 2,843,579, issued July 15, 1958, may be employed herein.

More particularly, the additive composition concentrates of our present invention are formed by neutralizing a hydrolyzed phosphorus sulfide-hydrocarbon reaction product, formed, for example, as indicated above and preferably solvent extracted, with an amine compound having 2 or more carbon atoms and preferably an aliphatic polyamine as defined above. The neutralized product is then reacted with difluoroboric acid preferably in amounts corresponding to from about 1 to about 3 moles boron per mole of neutralized product. We add up to about 1.1 moles of amine compound per mole of acid phosphorous in the hydrolyzed reaction product depending on the type of amine compound used. It is preferred to neutralize only one amine group of a given amine compound and, therefore, from about 1 to about 1.1 moles of the amine compound per mole of

acid phosphorus is preferred. No solvent is necessary for the reaction since difluoroboric acid is a liquid which is sufficiently soluble in the reaction mixture. During the difluoroboric acid reaction, it may be advantageous

- 5 to stir the mixture of neutralized reaction product and difluoroboric acid and to warm the mixture for a short period of time, for example about one hour, to increase the solubility of the difluoroboric acid. The reaction mixture is then heated to a temperature above 100° C. 10 to strip off water and allow the reaction to go to completion. We have found that when water is not stripped off the reaction is reversible and will not go to completion due to the instability of the reaction product in the presence of water. During warming, the reaction mixture should not be heated to a temperature at which the amine is driven from the mixture. If temperatures higher than the boiling point of the amine are used means for retaining the amine, such as, for example, refluxing, should be employed. An alternative method of forming 15 the fluorine and boron-containing amine-neutralized reaction products which we have found acceptable is by first reacting the difluoroboric acid with the amine compound and then reacting the resulting product with the phosphorus sulfide-hydrocarbon reaction product.
- 20 25 30 35 40 45 50

- If the product should be hazy due to the presence of impurities, for example the presence of excess difluoroboric acid which has not reacted with the neutralized phosphorus sulfide hydrocarbon reaction product or has not dissolved therein, it may be desirable to filter the product through diatomaceous earth to obtain a suitably clear product. The products formed in the above boron reaction contain chemically bonded boron and fluorine.

- The additive composition, prepared in accordance with the preferred method set out above, may be used in 35 lubricating oils in varying amounts constituting minor proportions of the total lubricating composition. The amount of additive used should be in excess of 0.1 weight percent. The additive is effective in imparting improved detergency lubricating oils even when used in such small amounts as range from about 0.1 weight percent. However, it is preferred to add the additive composition to the lubricating oil in amounts of from about one weight percent to about 10 weight percent although much greater amounts even above 15 weight percent may be advantageously employed. The additive when used in a lubricating oil in an internal combustion engine was also found to suppress the octane requirement increase of the engine probably by entering the combustion chamber by the process of blow-by.

#### 50 HYDROLYZED INTERMEDIATE

A hydrolyzed phosphorus sulfide-hydrocarbon reaction product is prepared by reacting about 15.5 wt. percent  $P_2S_5$  with a butylene polymer having a molecular weight of about 750-800 at a temperature of about 450° F. in a nitrogen atmosphere. The reaction is continued for about five hours for product formation. The product has a phosphorus content of about 4.3% and a sulfur content of about 7.5%. The reaction product formed 55 is then hydrolyzed with steam at a temperature of about 300° F. to about 400° F. The hydrolyzed product was diluted, for ease of handling, to about a 60% concentrate with a solvent extracted Mid-Continent 5W mineral oil having a viscosity of about 38 SSU at 210° F. The product 60 was then contacted with clay (fuller's earth) and filtered to remove inorganic impurities. The resulting clay treated product was used as a starting material for the preparation of additives in subsequent examples.

65 As a specific embodiment of our invention, the following examples are given by way of illustration and are not intended as limitations to the invention.

#### Example I

70 75 2030 grams (1.24 moles) of the clay contacted hydrolyzed intermediate were reacted with 141 grams (1.36

moles, 1.1 moles per mole of intermediate) of diethylene-triamine and a basic salt was formed. The basic salt was treated with 253 grams (3 moles) of difluoroboric acid ( $H_3BO_2F_2$ ; B.P. 159° C.) with stirring at 100° C. for four hours and 1320 grams of solvent extracted Mid-Continent 5W mineral oil having a viscosity of about 38 SSU at 210° F. were then added. The reaction mixture was filtered through Celite. The filtrate was a bright, brown, oil-soluble product which had a boron content of 0.35 wt. percent, a nitrogen content of 1.35 wt. percent, a phosphorus content of 1.16 wt. percent and a fluorine content of 2.0 wt. percent.

*Example II*

2035 grams (1.24 moles) of the clay contacted hydrolyzed intermediate were reacted with 199 grams (1.36 moles, 1.1 moles per mole of intermediate) of triethylenetetramine and a basic salt was formed. The basic salt was treated with 296 grams (3.53 moles) of difluoroboric acid ( $H_3BO_2F_2$ ; B.P. 159° C.) with stirring at 100° C. for four hours and 1059 grams of solvent extracted Mid-Continent 5W mineral oil having a viscosity of about 38 SSU at 210° F. were then added. The reaction mixture was blown with nitrogen at 125° F. and filtered through Celite. The filtrate was a bright, brown, oil-soluble product which had a boron content of 0.78 wt. percent, a nitrogen content of 1.77 wt. percent, a phosphorus content of 1.23 wt. percent and a fluorine content of 2.7 wt. percent.

*Example III*

2000 grams (1.22 moles) of the clay contacted hydrolyzed intermediate were reacted with 537 grams (1.34 moles, 1.1 moles per mole of intermediate) of Duomeen T and a basic salt was formed. Duomeen T commercially prepared by Armour Chemical Division, Chicago, Illinois, is predominantly a propylene diamine having a side chain derived from tallow-fatty acid and melting in the range of from about 44° C. to about 48° C.; the side chain is attached directly to the one nitrogen atom. The basic salt was treated with 125 grams (1.49 moles) of difluoroboric acid ( $H_3BO_2F_2$ ; B.P. 159° C.) with stirring at 100° C. for four hours and the reactants were then diluted with solvent extracted Mid-Continent 5W mineral oil having a viscosity of about 38 SSU at 210° F. and filtered through Celite. The filtrate was a bright, brown, oil-soluble product which had a boron content of 0.66 wt. percent, a nitrogen content of 1.02 wt. percent, a phosphorus content of 1.62 wt. percent and a fluorine content of 0.92 wt. percent.

The effectiveness of the products of the present invention in improving the detergency characteristics of lubricating oils is demonstrated by the data in Table I. The data were obtained by subjecting a commercial-type lubricating oil with and without the product of the above example to the detergency and oxidation test known as the Squalene Indiana Stirring Oxidation Test (I.S.O.T.). In the Squalene I.S.O.T., 10% by weight of squalene (a highly unsaturated reactive hydrocarbon that polymerizes easily and forms a tightly adhering varnish during the test) is added to the oil to be tested and the mixture is heated at 300° F. in a 500 cc. glass beaker in the presence of 5 square inches of copper and 10 square inches of iron. Four glass rods of 6 mm. diameter are suspended in the oil which is stirred at about 1300 r.p.m. by means of a glass stirrer. After 72 hours the test is ended and varnish values are determined. Varnish values or ratings are based upon visual inspection of the glass rods, in which a rod free of any varnish deposit is given a rating of 10 while a badly coated rod is given a rating of 1. Rods having appearances between these extremes are given intermediate values. The following comparative samples were subjected to the Squalene I.S.O.T. with the results listed in Table I.

- 5 Sample A—A mixture of 5 weight and 10 weight solvent extracted base stock containing a polyisobutylene polymer viscosity improver and having a viscosity of about 62 SSU at 210° F. and 0.75 weight percent sulfurized dipentene corrosion inhibitor.
- 10 Sample B—Sample A containing 3.79 weight percent of the product of Example I.
- 15 Sample C—Sample A containing 3.93 weight percent of the product of Example II.

TABLE I

| Sample: | Varnish rating |
|---------|----------------|
| A       | 4 to 5         |
| B       | 10             |
| C       | 10             |

20 A composition of the present invention was comparatively subjected to a Detergency Screening Test which rates detergency by a determination of piston varnish deposits. The test was carried out in a current model Chevrolet Powerglide Engine operating for one hour at 500 r.p.m. and no load and for 6 subsequent hours at 2500 r.p.m. and a load of 45 B.H.P. The oil temperature for the first hour was 100° F., for the second and third hours was 165° F. and for the 4 remaining hours was 220° F. The water temperature for the first 3 hours was from 85 to 95° F. and for the remaining 4 hours was 170 to 180° F. Each 7 hours so constituted is regarded a cycle. For the Detergency Screening Tests, 4 cycles were run with a 4-hour rest between each cycle.

25 At the end of the 4 cycles, the pistons were examined for varnish and rated on a scale whereby pistons free of varnish are rated 10 and pistons having very heavy varnish are rated one. The following samples were subjected to the above test and the comparative results are indicated in Table II.

30 Sample A—A phenol extracted Mid-Continent base stock mineral oil having a viscosity of about 45 SSU at 210° F. containing 0.75 weight percent sulfurized dipentene corrosion inhibitor.

35 Sample B—4.2 weight percent of the product of Example III in Sample A.

40 Sample C—3.9 weight percent of a barium containing neutralized phosphorus pentasulfide-butylene polymer (mol wt. of about 750 to 800) reaction product<sup>1</sup> and 0.79 weight percent of sulfurized dipentene in a solvent extracted Mid-Continent mineral oil containing a polyisobutylene polymer viscosity index improver and having a viscosity of about 62 SSU at 210° F.

45 Sample D—6.6 weight percent of a barium-containing neutralized phosphorus pentasulfide-butylene polymer (mol wt. of about 750 to 800) reaction product<sup>1</sup> in Sample A.

TABLE II.—RESULTS OF DETERGENCY SCREENING TEST

| Sample: | Piston varnish rating |
|---------|-----------------------|
| A       | 5.3                   |
| B       | 8.9                   |
| C       | 7.2                   |
| D       | 7.4                   |

50 60 As can be seen from Table III, the composition of the present invention indicated as Sample B gave superior piston varnish rating results in comparison with metal-containing detergent additives as exemplified by Samples C and D when compounded in commercial-type lubricants and also gave superior results in comparison with the very low piston varnish rating of the lubricant without any detergent additive as exemplified by Sample A.

65 70 The herein described additive compositions of the present invention can be used as indicated above in varying amounts of from 0.1 up to about 15 percent in lubri-

<sup>1</sup> For comparison of metal-containing phosphorus sulfide-hydrocarbon reaction products with the amine-containing fluoroboric acid complexes.

cating oils. Although the present invention has been illustrated by the use of the additive compositions in mineral lubricating oils, it is not restricted thereto. Other lubricating oil bases can be used, such as hydrocarbon oils, both natural and synthetic, for example, those obtained by the polymerization of olefins, as well as synthetic lubricating oils of the alkylene oxide type and the polycarboxylic acid ester type, such as the oil soluble esters of adipic acid, sebacic acid, azelaic acid, etc. It is also contemplated that various other well known additives, such as antioxidants, anti-foaming agents, pourpoint depressors, extreme pressure agents, antiwear agents, may be incorporated in lubricating oils containing the additives of our invention.

Concentrates of a suitable oil base containing more than 10 percent, for example up to 50 percent or more, of the additives of this invention alone or in combination with other additives can be used for blending with hydrocarbon oils or other oils in the proportions desired for the particular conditions of use to give a finished lubricating product containing the additives of this invention.

Unless otherwise stated, the percentages given herein and in the claims are percentages by weight.

Although we have described our invention by reference to specific embodiments and examples thereof, such specific embodiments and examples as have been given are merely for the purpose of illustration of the invention and are not intended as limiting its scope. It is intended that modifications and variations of the present inventions which are apparent from our foregoing description to those skilled in the art are to be considered within the scope of our present invention except as stated in the following appended claims.

We claim:

1. As a new composition of matter, an oil-soluble detergent neutralized reaction product prepared by the process comprising: reacting a phosphorus sulfide with a hydrocarbon; hydrolyzing the resulting phosphorus sulfide-hydrocarbon reaction product; and reacting the hydrolyzed product with fluoroboric acid in an amount corresponding to from about one to about three moles of boron per mole of reaction product and an aliphatic polyamine having from 2 to 21 carbon atoms in the aliphatic group in an amount corresponding to from about one to about 1.1 moles of polyamine per mole of acid phosphorus, at a temperature below the temperature at which said polyamine is driven from the mixture of reactants.

2. A lubricating composition comprising a major amount of hydrocarbon lubricating oil and from about 0.1 to about 20 weight percent of the composition of claim 1.

3. The composition of claim 1 wherein the aliphatic polyamine is diethylenetriamine.

4. The composition of claim 1 wherein the aliphatic polyamine is a propylene diamine having a side chain derived from taliof-fatty acid and melting in the range of 44° to 48° C.

5. The composition of claim 1 wherein the aliphatic polyamine is triethylene tetramine.

6. As a new composition of matter, an oil-soluble detergent neutralized reaction product prepared by the process comprising the steps of: reacting a phosphorus sulfide with a hydrocarbon; hydrolyzing the resultant phosphorus sulfide-hydrocarbon reaction product; neutralizing the hydrolyzed product with an aliphatic polyamine having from 2 to 21 carbon atoms in the aliphatic group in an amount corresponding to from about one to about 1.1 moles of polyamine per mole of acid phosphorus; and reacting the neutralized product with fluoroboric acid in an amount corresponding to from about one to about three moles of boron per mole of reaction product at a temperature below the temperature at which said polyamine is driven from the mixture of reactants.

7. A lubricating composition comprising a major amount of hydrocarbon lubricating oil and from about 0.1 to about 20 weight percent of the composition of claim 6.

8. As a new composition of matter, an oil-soluble detergent neutralized reaction product prepared by the process comprising the steps of: reacting a phosphorus sulfide with a hydrocarbon; hydrolyzing the resultant phosphorus sulfide-hydrocarbon reaction product; reacting fluoroboric acid in an amount corresponding to from about one to about three moles of boron per mole of reaction product with an aliphatic polyamine having from 2 to 21 carbon atoms in the alkylene group and containing at least two primary amino nitrogen atoms in an amount corresponding to from about one to about 1.1 moles of polyamine per mole of acid phosphorus; and reacting the resulting reaction product with a hydrolyzed phosphorus sulfide-hydrocarbon reaction product at a temperature below the temperature at which the polyamine is driven from the mixture of reactants.

9. As a new composition of matter, an oil-soluble detergent neutralized reaction product prepared by the process comprising the steps of: reacting phosphorus sulfide with a hydrocarbon; hydrolyzing the resulting phosphorus sulfide-hydrocarbon reaction product; neutralizing the resulting hydrolyzed product with from about one to about 1.1 moles of ethylene diamine per mole of hydrolyzed reaction product; and reacting the resulting neutralized product with from about one to about three moles based on boron of fluoroboric acid per mole of neutralized product at a temperature below the temperature at which the ethylene diamine is driven from the mixture of reactants.

10. As a new composition of matter, an oil-soluble detergent neutralized reaction product prepared by the process comprising the steps of: reacting phosphorus sulfide with a butene polymer at a temperature of from about 200° F. to about 600° F.; hydrolyzing the resulting phosphorus sulfide-butene polymer reaction product; neutralizing the resulting hydrolyzed product with from about one to about 1.1 moles per mole of hydrolyzed reaction product of an alkylene polyamine having the formula  $RNH(CH_2)_3NH_2$  wherein R is a  $C_{10}$  to  $C_{18}$  aliphatic chain; reacting the resulting neutralized product with from about one to about three moles based on boron of fluoroboric acid per mole of neutralized product at a temperature below the temperature at which the polyamine is driven from the mixture of reactants; and heating the reactants to a temperature above 100° C. whereby water is stripped from the reaction mixture.

11. A lubricant additive concentrate consisting essentially of a hydrocarbon lubricating oil containing more than about 10% of an oil-soluble detergent neutralized reaction product prepared by the process comprising: reacting a phosphorus sulfide with a hydrocarbon; hydrolyzing the resulting phosphorus sulfide-hydrocarbon reaction product; and reacting the hydrolyzed product with fluoroboric acid in an amount corresponding to from about one to about three moles of boron per mole of reaction product and an aliphatic polyamine having from 2 to 21 carbon atoms in the aliphatic group in an amount corresponding to from about one to about 1.1 moles of polyamine per mole of acid phosphorus, at a temperature below the temperature at which the polyamine is driven from the mixture of reactants.

12. A lubricant additive concentrate consisting essentially of a hydrocarbon lubricating oil containing more than about 10% of an oil-soluble detergent neutralized reaction product prepared by the process comprising: reacting a phosphorus sulfide with a hydrocarbon; hydrolyzing the resulting phosphorus sulfide-hydrocarbon reaction product; and reacting the hydrolyzed product with fluoroboric acid in an amount corresponding to from about one to about three moles of boron per mole of reaction product and an aliphatic polyamine having from 2 to 21 carbon atoms in the aliphatic group in an amount corresponding to from about one to about 1.1 moles of polyamine per mole of acid phosphorus, at a temperature below the temperature at which the polyamine is driven from the mixture of reactants.

#### References Cited in the file of this patent

#### UNITED STATES PATENTS

- |    |           |                         |               |
|----|-----------|-------------------------|---------------|
| 70 | 2,053,474 | Graves et al. -----     | Sept. 8, 1936 |
|    | 2,160,917 | Shoemaker et al. -----  | June 6, 1939  |
|    | 2,346,156 | Farrington et al. ----- | Apr. 11, 1944 |
|    | 2,636,858 | Jones et al. -----      | Apr. 28, 1953 |
|    | 2,798,045 | Buck et al. -----       | July 2, 1957  |
|    | 2,809,934 | Alford et al. -----     | Oct. 15, 1957 |
| 75 | 2,900,376 | Sabol et al. -----      | Aug. 18, 1959 |